

April 23, 1935.

W. S. JONES

1,998,506

MOUNTING FOR LEAF AND POWDERED METALS

Filed Dec. 2, 1931

*Fig. 1.*



*Fig. 2.*



*Fig. 3.*



*Fig. 4.*



*Fig. 6.*

INVENTOR.  
WILLIAM S. JONES.

BY  
Kiddle, Mangeson and Horridge.  
ATTORNEYS.

## UNITED STATES PATENT OFFICE

1,998,506

## MOUNTING FOR LEAF AND POWDERED METALS

William S. Jones, Windsor, Conn.

Application December 2, 1931; Serial No. 578,515

2 Claims. (Cl. 91—68)

My invention relates to a new and novel mounting for gold or other precious metals in leaf or powdered form particularly adapting the same for use in heat embossing for the ornamentation of leather, cloth and other materials.

Heretofore it has been customary to mount gold or other precious metal in leaf form upon a sheet or ribbon or tape of paper, attaching the metal to the paper by suitable adhesive such as wax.

10 After the metal leaf is secured to the sheet or ribbon of paper, as the case may be, then a suitable size, such as French varnish, may be applied to the surface of the metal. When heat and pressure are applied by a die to a strip or sheet of material so prepared the adhesive will be melted and permit the paper to be separated from the metal leaf, the size causing the leaf to adhere to the surface being ornamented. On the other hand the size may be applied directly to the surface of the material to be ornamented instead of to the surface of the metal leaf.

It has also been customary to mount various metals such as aluminum, bronze and other metals in powdered form on paper sheets or ribbons or tapes by means of a suitable adhesive. After the surplus powder which does not adhere to the paper has been removed then a suitable size is usually sprayed upon the powdered surface. This enables a powdered metal to be affixed to leather, cloth or other surfaces by means of a heated die as in the case of metal leaf.

One of the objects of my invention is to mount metal leaf or metallic powder upon a support of metal foil, such as tin, lead, aluminum, etc., preferably aluminum foil, as I have found that the use of metal foil by reason of its heat conducting and non-absorbent characteristics will greatly enhance the burnishing effect of the metal leaf and also of the metallic powder to be applied to an embossed surface.

Another object of my invention is to provide a suitable supporting or carrying medium for metal leaf or metallic powder that is not destroyed during the burnishing operation but can be reclaimed and used again.

Other objects of my invention will appear from the detailed description that follows in which:

Fig. 1 illustrates metal leaf applied directly to a sheet of metal foil;

Fig. 2 illustrates an embodiment of my invention in which a sheet of metal leaf is attached to a sheet of metal foil by an adhesive;

Fig. 3 illustrates an embodiment of my invention in which metal powder is attached to a sheet of metal foil by an adhesive;

Fig. 4 illustrates a roll of metal foil in ribbon form with metal leaf secured directly thereto;

Fig. 5 illustrates a roll of metal foil in which metal leaf is secured thereto by an adhesive; and

Fig. 6 illustrates a roll of metal foil in ribbon form in which a metallic powder is attached thereto by means of an adhesive.

Referring to the drawing and first of all to Fig. 1, A represents a thin sheet of metal foil, preferably aluminum foil. This foil is of substantially the same thickness as that of paper upon which gold leaf is usually mounted. To one surface of this sheet of metal foil is directly applied a sheet of gold leaf which is designated B. To the surface of this gold leaf is applied a suitable size, such as French varnish, and designated C. In use, as will be appreciated, the sized surface of the leaf is applied directly to the leather, cloth or other surface to be ornamented and a heated die applied to the back of the foil A. The heat of the die will cause the size to attach the leaf to the surface being ornamented whereupon the foil can be stripped or separated from the leaf and reclaimed.

I have found that the metal foil is very advantageous in this class of work in that it will not curl under heat and by reason of its heat conducting characteristic, being an excellent conductor of heat, will greatly enhance the burnishing effect on the metal leaf.

It will be appreciated that the use of this foil has a further advantage in that in the mounting of the leaf on the foil one step may be eliminated, that is to say, the step in which adhesive is applied to the foil for the purpose of attaching the leaf to the foil, the embodiment of my invention as illustrated in Fig. 1 mounting the leaf directly on the foil.

In Fig. 2 I have shown an embodiment of my invention similar to that illustrated in Fig. 1, employing the metal foil A, gold leaf B and size C. In this embodiment of my invention, however, I have shown an adhesive D for attaching the leaf to the foil. I have obtained good results employing sour milk as the adhesive D, although a material like paraffin gives fairly good results.

In the form of my invention illustrated in Fig. 3 one surface of the foil A is coated with a suitable adhesive D such as sour milk, for example, and on this adhesive I apply a metal powder E, such as aluminum, bronze and other metals, the surface of this powder having a size C such as French varnish, for instance, applied thereto.

In use, with reference to the two embodiments of my invention illustrated in Figs. 2 and 3, a hot

die is applied to the outer surface of the foil A as before, the heat of the die not only burnishing the leaf B or the powder E, as the case may be, but causing the leaf or the powder to adhere to the surface of the material being ornamented, the heat of the die also permitting of ready separation of the foil A from the leaf or the powder, as the case may be.

I find when employing an adhesive between 10 the metal and the foil that the non-absorbent characteristic of the foil is advantageous, the metal adhering to the foil more satisfactorily than when employing a backing or mounting, such as paper for instance, commonly employed 15 in this art.

In Fig. 4 I have illustrated the foil F in ribbon form as distinguished from the sheet form of Figs. 1 to 3. The metal leaf G is mounted directly on one side of this foil and the surface of 20 this metal leaf coated with the size H as in Fig. 1, for instance.

In Fig. 5 I employ foil F in ribbon form, the surface of this foil being coated with an adhesive 25 I for attaching leaf G in ribbon form to the foil, the surface of the leaf G being coated with a suitable size H.

Fig. 6 is similar to Fig. 5 except that the leaf G has been substituted by a metal powder J, the surface of this powder being coated with suitable size H.

While I have pointed out in the various embodiments of my invention that a size is applied to the outer surface of the leaf or powder mounted upon the foil it is to be understood that if desired the size may be applied to the surface to be ornamented.

It will be appreciated that in use the foil will not be destroyed by the die as in the case of paper mountings but can be reclaimed, thereby avoiding the waste present when paper mountings are used.

What I claim is:—

1. As an article of manufacture for heat embossing thin aluminum foil having a surface coated with metallic powder secured thereto by a suitable adhesive.

2. As an article of manufacture for heat embossing thin aluminum foil having a surface coated with metallic powder secured thereto by a suitable adhesive, the powdered surface having a coating of a suitable size.

WILLIAM S. JONES.